



US005320867A

# United States Patent [19]

Bachot et al.

[11] Patent Number: 5,320,867  
[45] Date of Patent: Jun. 14, 1994

[54] **METHOD OF MAKING MICROPOROUS ASBESTOS DIAPHRAGMS/CATHODES FOR ELECTROLYTIC CELLS**

[75] Inventors: **Jean Bachot, Bourg la Reine; Pascal Stutzmann, Paris; Jean-Maurice Perineau, Claix, all of France**

[73] Assignee: **Rhone-Poulenc Chimie, Courbevoie, France**

[21] Appl. No.: **802,319**

[22] Filed: **Dec. 4, 1991**

## Related U.S. Application Data

[62] Division of Ser. No. 565,344, Aug. 10, 1990, Pat. No. 5,092,977.

## Foreign Application Priority Data

Aug. 10, 1989 [FR] France ..... 89 10937

[51] Int. Cl.<sup>5</sup> ..... **B05D 3/02**

[52] U.S. Cl. ..... **427/226; 427/246; 427/294; 427/77; 432/13; 204/296; 204/282**

[58] Field of Search ..... **204/295, 296, 282; 427/77, 245, 58, 226, 126.3, 294, 246; 432/13**

## References Cited

### U.S. PATENT DOCUMENTS

3,980,613 9/1976 Bachot et al. ..... 264/415.3  
4,105,516 8/1978 Martinsons et al. ..... 204/129  
4,354,900 10/1982 Bailey et al. ..... 162/106  
4,410,411 10/1983 Fenn, III et al. ..... 204/283  
4,447,566 5/1984 Hruska et al. ..... 523/221  
4,563,260 1/1986 Hruska et al. ..... 204/253  
4,665,120 5/1987 Hruska et al. ..... 524/452

4,701,250 10/1987 Fenn, III et al. ..... 204/283  
4,720,334 1/1988 DuBois et al. ..... 204/296  
4,743,349 5/1988 Bachot et al. ..... 204/242  
4,775,551 10/1988 Bachot et al. ..... 427/58  
4,810,345 3/1989 Schulz et al. ..... 264/295  
4,939,028 7/1990 Bachot et al. ..... 428/311.5  
4,940,524 7/1990 Perineau et al. ..... 204/242  
5,023,127 6/1991 Bachot ..... 428/137

## FOREIGN PATENT DOCUMENTS

0132425 1/1985 European Pat. Off. .... C25B 11/04  
0214066 3/1987 European Pat. Off. .... C25B 11/12  
0296076 12/1988 European Pat. Off. .... C25B 11/04  
2213805 8/1974 France ..... B01K 3/10  
2229739 12/1974 France ..... C08J 1/34

Primary Examiner—Kathryn Gorgos

Attorney, Agent, or Firm—Burns, Doane, Swecker & Mathis

## [57] ABSTRACT

Microporous diaphragms adapted for wet-consolidation with composite cathodes for use in electrolytic cells, e.g., chlorine/soda electrolysis cells, comprise a sintered, fluoropolymer microconsolidated asbestos-based microporous fibrous sheet material, such sheet material including from 3% to 35% by weight of fluoropolymer binder, from 1% to 50% by weight of a uniformly distributed gel of an oxohydroxide of at least one metal of Groups IVA, IVB, VB and VIB of the Periodic Table or of the lanthanide or actinide series thereof, and from 20% to 95% by weight of fibers, at least 1% by weight of such fibers being asbestos fibers.

14 Claims, No Drawings

**METHOD OF MAKING MICROPOROUS  
ASBESTOS DIAPHRAGMS/CATHODES FOR  
ELECTROLYTIC CELLS**

This application is a divisional, of application Ser. No. 07/565,344, filed Aug. 10, 1990, now U.S. Pat. No. 5,092,977.

**CROSS-REFERENCE TO COMPANION  
APPLICATION**

Copending application Ser. No. 07/565,385, now abandoned, filed concurrently herewith and assigned to the assignee hereof.

**BACKGROUND OF THE INVENTION**

**1. Field of the Invention**

The present invention relates to novel diaphragms comprising asbestos fibers adapted for use in electrolytic cells, to the coupling of such diaphragms with a cathode component of such cells and to a process for producing such diaphragms and coupling such diaphragms with a cathode component.

This invention especially relates to improved diaphragms produced via a wet route, based on asbestos fibers, and adapted for use in chlorine/soda electrolysis cells.

**2. Description of the Prior Art**

Asbestos fibers have long been employed in this art as a conventional material for producing the diaphragms used in electrolytic cells. These diaphragms are fabricated by depositing asbestos fibers contained in an aqueous mash onto a cathode which is permeable to the electrolytes, the deposition operation being carried out under vacuum. Thus, French Patent No. 2,213,805 describes preparing microporous separators by depositing a layer of asbestos, said layer being consolidated by a fluoropolymer. The porosity of such a layer can be better controlled by adding a pore-forming agent according to the technique described in French Patent No. 2,229,739.

As is well known to this art, such preparation of microporous separators by depositing, under vacuum, an aqueous mash containing fibers and a binder presents a very great advantage, both from a technological standpoint, as well as from an economic standpoint. However, the quality of the separators thus produced is not fully satisfactory.

Indeed, the Faraday yield is insufficient, and this is reflected in a high energy consumption per ton of chlorine produced. The higher the sodium hydroxide concentration, the more the yield in question is lowered on an industrial level. Thus, it is of the greatest importance to be able to operate with concentrated sodium hydroxide, in order to reduce the energy cost of the evaporation which is subsequently required to concentrate the sodium hydroxide produced. It would, therefore, be desirable to provide an improved diaphragm based on asbestos fibers and capable of being produced by a wet route.

In published European Patent Application No. 132,425 cathode components have been described, composite material produced by the coupling of an elementary cathode including a highly porous metal surface such as a metal grid having a mesh opening ranging from 20  $\mu\text{m}$  to 5 mm and of a sheet containing fibers and a binder, the coupling and the sheet resulting from the programmed suction under vacuum of a suspension

containing essentially electrically conductive fibers and a fluoropolymer, directly through said elementary cathode, followed by drying, and then melting the binder. Such composite materials that are adapted to themselves constitute the cathode of an electrolysis cell and may be coupled with a diaphragm, it being possible for the diaphragm to be manufactured directly by a wet route on the composite.

Various improvements have also been made, both to 10 the composite materials themselves, as well as to the process for the manufacture thereof.

In published European Patent Application No. 214,066 materials are described, containing carbon fibers exhibiting a monodisperse length distribution, materials whose quality and properties are very appreciably improved, and this is reflected in a much more favorable performance/thickness relationship.

In published European Patent Application No. 296,076 electroactivated materials are described which 20 contain an electrocatalytic agent uniformly distributed within their bulk mass, said agent being selected from among Raney metals and Raney alloys from which most of the easily removable metal(s) has (have) been removed.

The assemblage of proposed cathode components which ensure an appreciable distribution of the current is adapted for use in an electrolytic cell which will comprise a membrane or a diaphragm between the anode and cathode compartments. Additional technical 30 details are described in the aforementioned European patent applications, hereby expressly incorporated by reference in respect of the construction of said cathode components.

**SUMMARY OF THE INVENTION**

A major object of the present invention is the provision of improved microporous separators comprising asbestos fibers by a wet route, by vacuum suction of an aqueous mash containing asbestos fibers through a porous support, which improved microporous separators conspicuously ameliorate those disadvantages and drawbacks to date characterizing the state of this art.

Briefly, the present invention features novel microporous diaphragms that can be produced in situ by a wet route, comprising a fibrous sheet containing asbestos fibers that have been microconsolidated by a fluoropolymer, said sheet having been sintered and comprising:

- 50 (i) from 3% to 35% by weight of a fluoropolymer, binding the fibers;
- (ii) from 1% to 50% by weight of a gel of an oxohydroxide of at least one metal of Groups IVA, IVB, VB and VIB of the Periodic Table or of the lanthanide and actinide series; and
- (iii) from 20% to 95% by weight of fibers, at least 1% by weight of such fibers being asbestos fibers.

The present invention also features the coupling of the above novel diaphragms to a composite cathode component.

60 This invention also features a process for the production of such diaphragms, comprising the following sequence of stages:

- (a) preparing, in an essentially aqueous medium, a dispersion comprising the fibers, the fluoropolymer-based binder in the form of particles, if appropriate at least one precursor of an oxohydroxide of at least one of the metals of Groups IVA, IVB, VB and VIB of the Periodic Table or of the lanthanide

- and actinide series, also in particle form, and, if appropriate, additives;
- (b) depositing a sheet by programmed vacuum filtration of said dispersion through a porous support material;
  - (c) removing the liquid medium and, if appropriate, drying the sheet thus formed;
  - (d) sintering this sheet; and
  - (e) treating, if appropriate, in situ under the conditions of electrolysis, the sintered sheet with an aqueous solution of an alkali metal hydroxide.

The porous material (support) may then constitute a composite cathode component, and the above process then enables producing a coupling according to the present invention.

Thus, the present invention also features a process for the preparation of such couplings comprising the following sequence of stages:

- (a) depositing a precathodic sheet by programmed vacuum filtration of a dispersion, in an essentially aqueous medium, of fibers, of particulate binder and, if appropriate, of additives, through an elementary cathode which comprises a metal surface having mesh openings or perforations ranging from 20  $\mu\text{m}$  to 5 mm;
- (b) removing the liquid medium and, where appropriate, drying the sheet thus formed;
- (c) programmed vacuum filtering, through the precathodic sheet, of a dispersion, in an essentially aqueous medium, of fibers, of particulate binder based on a fluoropolymer, of at least one precursor of an oxohydroxide of at least one of the metals of Groups IVA, IVB, VB and VIB of the Periodic Table or of the lanthanide and actinide series, in the form of particles, and, if appropriate, of additives;
- (d) removing the liquid medium and, where appropriate, drying the sheet thus formed;
- (e) sintering of such sheet; and
- (f) treating, if appropriate in situ under the conditions of the electrolysis, such sintered sheet with an aqueous solution of an alkali metal hydroxide.

#### DETAILED DESCRIPTION OF THE PREFERRED EMBODIMENTS OF THE INVENTION

More particularly according to the present invention, the subject novel diaphragms exhibit an appreciable dimensional stability, a fine and uniform porosity and a permanent wettability. The diaphragms according to the present invention additionally exhibit very low operating voltages, and this constitutes another advantage of this invention.

The diaphragms according to the present invention are advantageously produced by the routes, traditionally employed industrially, of deposition of a suspension by suction under vacuum, and permit the efficient (high current yield) operation of brine electrolysis cells comprising same, at high current densities which can extend up to 40  $\text{A}/\text{dm}^2$  and higher. Moreover, such diaphragms permit cell operation at high sodium hydroxide concentrations (on the order of 140 to 200 g/l or higher) in the catholyte, and this limits the energy consumption required for the subsequent concentration of sodium hydroxide.

The diaphragms according to the invention comprise an asbestos-based fibrous sheet. By "sheet" is intended a three-dimensional assembly or stack whose thickness is appreciably smaller than its other dimensions, it being

possible for said assembly, if appropriate, to have two parallel face surfaces. These sheets can be in various forms, generally determined by the geometry of the cathode components with which they may later be coupled. In their use as microporous diaphragms in cells for the electrolysis of sodium chloride, and by way of example, their thickness typically ranges from 0.1 to 5 mm, and one of their long dimensions, corresponding substantially to the height of the cathode component, can extend up to 1 m or even more, and the other long dimension, reflecting substantially the perimeter of the component in question, can extend up to several tens of meters.

The fibers of the sheet are microconsolidated, namely, they are, in a fashion, attached or interconnected to each other, above all, by a three-dimensional network of discrete bonding points, and this contributes to ensuring that the sheet has a porosity which is at the same time fine and uniform, and a very great cohesion.

These sheets (or fibrous stacks) according to the invention are based on asbestos and essentially consist of, as indicated above:

- (i) from 3% to 35% by weight of a fluoropolymer binder;
- (ii) from 1% to 50% by weight of a gel of an oxohydroxide of at least one metal of Groups IVA, IVB, VB and VIB of the Periodic Table or of the lanthanide and actinide series; and
- (iii) from 20% to 95% by weight of fibers, at least 1% by weight of said fibers being asbestos fibers.

By "fluoropolymer" is intended a homopolymer or a copolymer derived at least partly from olefinic monomers completely substituted by fluorine atoms or completely substituted by a combination of fluorine atoms and of at least one of chlorine, bromine or iodine atoms per monomer.

Exemplary fluoro homo- or copolymers include polymers and copolymers derived from tetrafluoroethylene, hexafluoropropylene, chlorotrifluoroethylene and bromotrifluoroethylene.

Such fluoropolymers may also contain up to 75 mole percent of recurring structural units derived from other ethylenically unsaturated monomers containing at least as many fluorine atoms as carbon atoms, such as, for example, vinylidene (di)fluoride, or vinyl perfluoroalkyl ethers such as perfluoroalkoxyethylene.

A plurality of fluoro homo- or copolymers such as described above can, of course, be used according to the present invention. It, too, will be appreciated that it is also within the scope of this invention to use together with these fluoropolymers a small quantity, for example up to 10% or 15% by weight of polymers that do not contain fluorine atoms, such as, for example, polypropylene.

Polytetrafluoroethylene is the preferred binder of the diaphragms according to the invention.

The fluoropolymer employed as the binder for the assembly of fibers may be present in the subject diaphragms in amounts which can vary over wide limits, bearing in mind the fiber content and the nature of the various constituents of such diaphragms.

However, to ensure a good consolidation of the assembly, the binder will preferably constitute from 5% to 40% by weight in the subassembly (fibers + binder).

The diaphragms according to the invention also comprise from 20% to 95% by weight of fibers.

These fibers, of which at least 1% (by weight) and, preferably at least 40% (by weight) are asbestos fibers,

can be of various types. It is possible, indeed, to use different inorganic fibers, organic fibers, or mixtures of inorganic fibers and organic fibers. Exemplary organic fibers for forming the diaphragms according to the present invention include fibers of the fluoropolymers indicated above and, more particularly, polytetrafluoroethylene (PTFE) fibers.

The PTFE fibers according to the present invention may be of variable sizes; their diameter (D) typically ranges from 10 to 500  $\mu\text{m}$  and their length (L) is such that the ratio (L/D) advantageously ranges from 5 to 500. Those preferred are PTFE fibers having mean dimensions ranging from 1 to 4 mm in the case of length and ranging from 50 to 200  $\mu\text{m}$  in the case of diameter. Their preparation is described in U.S. Pat. No. 4,444,640 and PTFE fibers of this type are known to the art.

Exemplary inorganic fibers for forming the diaphragms according to the present invention include zirconia, carbon, graphite or titanate fibers.

The carbon or graphite fibers are in the form of filaments whose diameter is generally smaller than 1 mm and preferably ranges from  $10^{-5}$  to 0.1 mm and whose length is greater than 0.5 mm and preferably ranges from 1 to 20 mm.

These carbon or graphite fibers preferably have a monodisperse length distribution, namely, a distribution of lengths such that the length of at least 80%, and advantageously of at least 90%, of the fibers is within  $\pm 20\%$ , and preferably within  $\pm 10\%$ , of the average length of the fibers. When they are present, these carbon fibers advantageously constitute not more than 10% by weight of the combined fibers.

The titanate fibers are fibrous materials which are known per se. Thus, potassium titanate fibers are available commercially. Other suitable fibers are those derived from potassium octatitanate  $\text{K}_2\text{Ti}_8\text{O}_{17}$  by partial replacement of the ions of titanium in the oxidation state of IV with metal cations in the oxidation state of II, such as magnesium and nickel cations, or in the oxidation state of III, such as iron or chromium cations, and displaying charge compensation ensured by alkali metal ions such as sodium and potassium cations. These are described in published French Patent Application No. 2,555,207.

Other titanate fibers, such as those of potassium tetratitanate ( $\text{K}_2\text{Ti}_4\text{O}_9$ ) or those derived therefrom, can also be employed. While the titanate fibers can, without major inconvenience, constitute up to 80% by weight of the fiber mixture employed, it is preferable, when using carbon or graphite fibers, that their proportion in the fiber mixture should not exceed 10% by weight.

Mixtures of inorganic fibers which differ in their nature can, of course, also be employed.

The diaphragms according to the invention also contain from 1% to 50% by weight of a gel of an oxohydroxide of at least one metal of Groups IVA, IVB, VB and VIB of the Periodic Table or of the lanthanide and actinide series. The gel content preferably constitutes from 2% to 25% by weight and, more preferably, at least 3% by weight.

This gel is distributed uniformly both at the surface of the diaphragms according to the invention and into the depth thereof.

The content of gel, initially impregnated with sodium chloride, sodium hydroxide and water, is determined after contact at 85° C. with an aqueous solution containing 140 g/l of sodium hydroxide and 160 g/l of sodium

chloride, followed by cooling to 25° C., washing with water and drying for 24 hours at 100° C.

Examples of the metals of the Groups and series of the Periodic Table which are noted above which are representative are titanium, zirconium, thorium, cerium, tin, tantalum, niobium, uranium, chromium and iron. Mixtures of such metals or of such metals and of alkali metals such as sodium or potassium may, of course, be present in the diaphragms according to the invention.

The diaphragms according to the invention preferably contain a gel of an oxohydroxide of at least one metal of Groups IVA and IVB.

They preferably contain a titanium, zirconium or cerium oxohydroxide gel.

The diaphragms according to this invention have been defined in terms of their essential constituents. It will be appreciated that these materials can contain various other additives in a minor amount generally not exceeding 5% by weight, which will have been added either simultaneously or successively during any of the stages of their production. Thus, they can contain trace amounts of surface-active or surfactant agents, of pore-forming agents whose function is to regulate the porosity of the diaphragm, and/or of thickeners, although such agents are in principle decomposed or removed during the production of the said diaphragm.

The diaphragms according to the present invention advantageously have a weight per unit of surface area ranging from 0.4 to 3  $\text{kg}/\text{m}^2$  and preferably from 0.7 to 1.9  $\text{kg}/\text{m}^2$ .

The present invention also features the coupling of a composite cathode component and of a diaphragm as described above.

These composite cathode (or precathodic) components are produced by the coupling of an elementary cathode comprising a highly porous metal surface and a microporous fibrous sheet containing a significant proportion of electrically conductive fibers, such fibers being microconsolidated by a fluoropolymer.

The preferred cathode (or precathodic) components according to the present invention contain carbon or graphite fibers as electrically conductive fibers. These fibers preferably have a monodisperse length distribution.

Although the fluoropolymer binder for the precathodic sheet may be selected from the fluoropolymers described above, polytetrafluoroethylene is the preferred.

These composite cathode (or precathodic) components are described in the European patent applications hereinbefore incorporated by reference.

It will be apparent that the coupling under consideration entails an assembly of one face surface towards the other of three layers, namely, the elementary cathode, a first fibrous sheet containing the electrically conductive fibers, such sheet having intrinsic properties which are described in said European patent applications, and the diaphragm, said assembly constituting a coherent complete organization.

Also as indicated above, the present invention also features a process for the production of the diaphragms described immediately above.

The process for the preparation of the subject diaphragms comprises the following sequence of stages:

(a) preparing, in an essentially aqueous medium, a dispersion comprising the fibers, the fluoropolymer-based binder in the form of particles, at least one precursor of an oxohydroxide of at least one of the

metals of Groups IVA, IVB, VB and VIB of the Periodic Table or of the lanthanide and actinide series, in the form of particles and, if appropriate, additives;

- (b) depositing a sheet by programmed vacuum filtration of said dispersion through a porous support material;
- (c) removing the liquid medium and, if appropriate, drying the sheet thus formed;
- (d) sintering such sheet; and
- (e) treating, if appropriate, *in situ* under the conditions of the electrolysis, such sintered sheet with an aqueous solution of alkali metal hydroxide.

By "essentially aqueous medium" is intended a medium containing no organic compounds other than the constituents indicated above and additives such as surface-active agents, surfactants and thickeners. Thus, the medium in question does not contain any organic solvent.

Indeed, while the presence of organic solvents is not detrimental in and of itself, one advantage presented both by the present process and the diaphragms according to the invention is the fact that the presence of organic solvents is not necessary for the production of such diaphragms and that, as a result, it is not necessary to provide an additional stage of evaporation of the solvent.

By "precursors of an oxohydroxide of one of the metals of Groups IVA, IVB, VB and VIB of the Periodic Table or of the lanthanide and actinide series" are intended salts of said metals, as poorly soluble as possible in water, in which the anion is advantageously selected from among the phosphate, pyrophosphate, hydrogen phosphate or polyphosphate anions, substituted where appropriate by an alkali metal, and silicate.

Exemplary salts which can be used according to the present process include:

- Titanium phosphate ( $\alpha$ -TiP)
- Zirconium phosphate ( $\alpha$ -ZrP)
- Cerium phosphate
- $Ti(NaPO_4)_2$
- $TiNaH(PO_4)_2$
- $TiP_2O_7$
- $TaH(PO_4)_2$
- $NbOPO_4$
- $UO_2HPO_4$
- $Cr_5(P_3O_{10})_3$
- $Fe_4(P_2O_7)_3$

The compounds corresponding to the formula



in which M is a sodium or lithium atom and x is a number which may be zero and smaller than 3.

These precursors are introduced in the form of particles. They may be introduced in the form of a powder having a particle size which is generally smaller than 500  $\mu m$  or in the form of fibers whose dimensions typically range from 0.1 to 50  $\mu m$  in the case of diameter and from 3  $\mu m$  to 3 mm in the case of length.

The fluoropolymer-based binder is typically in the form of a dry powder or of an aqueous dispersion (latex) whose solids content constitutes from 30% to 80% by weight.

As is well known to this art, the dispersion or suspension under consideration is generally highly dilute, the content of dry matter (fibers, binder, precursors and additives) representing on the order of 1% to 15% of

the weight of the entire mass, to make it easier to handle on an industrial scale.

Various additives may also be introduced into the dispersion, in particular surface-active agents or surfactants such as octoxynol (Triton X-100  $\circledR$ ), pore-forming agents such as silica, and thickening agents such as natural or synthetic polysaccharides.

The dispersion will obviously contain all of the essential constituents of the diaphragm with the exception of the oxohydroxide gel discussed above, but gel precursors as described above will be present.

The relative amounts of the essential constituents of the diaphragm to be introduced into the dispersion can be readily determined by one skilled in this art, in consideration of the fact that they are substantially the same as those present in the diaphragm itself, with the exceptions of the pore-former which is in principle removed by the action, for example, of the electrolytic sodium hydroxide and of the oxohydroxide gel precursor. Indeed, the precursor is completely converted into oxohydroxide gel in which the "active" part obtained after washing and drying the gel, constitutes from 10% to 90% by weight of the precursor introduced.

One skilled in this art can also easily determine, using simple tests, the amount of dry solids to be dispersed in the aqueous medium as a function of the degree of retention which can be observed on the porous material through which the dispersion is filtered under the programmed vacuum conditions.

In general, the solids content in suspension comprises, as the principal constituents:

- (i) from 30% to 80% by weight of fibers;
- (ii) from 1% to 50% by weight of at least one oxohydroxide gel precursor;
- (iii) from 5% to 35% by weight of PTFE powder (binder); and
- (iv) from 5% to 40% by weight of silica.

To satisfactorily carry out the present invention, the content of PTFE powder constitutes from 5% to 40% by weight of the entire mass (PTFE powder + fibers). Also to advantageously carry out the present invention, the weight content of at least one oxohydroxide gel precursor in said solids content will range from 5% to 40%.

The sheet is then formed by programmed vacuum filtration of the dispersion through a porous material such as cloths or grids in which the mesh opening, the perforations or the porosity, advantageously ranges from 1  $\mu m$  to 2 mm.

The vacuum program may be continuous or stage-wise, from atmospheric pressure to the final pressure (0.01 to 0.5 bars absolute).

After removal of the liquid medium and, where appropriate, the drying of the sheet thus obtained, the sheet is sintered.

The sintering is carried out in a manner known per se at a temperature above the melting or softening point of the fluoropolymer binding the sheet. This stage, which permits the sheet to be consolidated, is then followed by a stage of treatment, by means of which the sheet is contacted with an aqueous solution of alkali metal hydroxide, and more particularly with an electrolytic sodium hydroxide solution.

This contacting may be conducted *in situ*, namely, when the consolidated sheet is placed in the electrolytic cell, in contact with the electrolytic sodium hydroxide solution.

The contacting is advantageously carried out with an aqueous solution of sodium hydroxide, the concentration of which ranges from 40% to 200 g/l and at a temperature ranging from 20° to 95° C.

The precursors of the oxohydroxide gel, described above, are capable of undergoing various conversions during the various operations of production of the diaphragm, and especially a nondestructive conversion during the sintering operation, i.e., resulting solely in losses of molecules of water of hydration or of formation; they will be converted by the aforementioned treatment stage into a fresh gel of oxohydroxide of the metal in question, impregnated with electrolyte and with water.

The properties of a diaphragm of this type are markedly improved.

Moreover, using precursors in the form of powder renders the processing considerably easier.

In a preferred alternate embodiment of the invention, the filtration of the dispersion or suspension is carried out through a cathode (or precathodic) component as defined above.

Such alternate embodiment enables production of a diaphragm/precathodic component coupling.

Such a coupling exhibits remarkable coherence properties, linking together the advantages presented by the precathodic component and the diaphragms according to the invention.

This invention also features a process for the preparation of such couplings, comprising the following sequence of stages:

- (a) depositing a precathodic sheet by programmed vacuum filtration of a dispersion, in an essentially aqueous medium, of fibers, of binder in the form of particles and, if appropriate, of additives, through an elementary cathode which comprises a metal surface exhibiting a mesh opening or perforations ranging from 20  $\mu\text{m}$  to 5 mm;
- (b) removing the liquid medium and, where appropriate, drying the sheet thus formed;
- (c) programmed vacuum filtering, through the precathodic sheet, of a dispersion, in an essentially aqueous medium, of fibers, of binder based on a fluoropolymer in the form of particles, of at least one precursor of an oxohydroxide of at least one of the metals of Groups IVA, IVB, VB and VIB of the Periodic Table or of the lanthanide and actinide series, in the form of particles and, where appropriate, of additives;
- (d) removing the liquid medium and, where appropriate, drying the sheet thus formed;
- (e) sintering of the resulting sheet; and
- (f) treating, if appropriate in situ under the conditions of the electrolysis, the sintered sheet with an aqueous solution of alkali metal hydroxide.

Such a process presents the advantage of contributing to establishing couplings of great cohesion. Another advantage is its great simplicity of implementation due to the fact that a single sintering stage is sufficient to produce couplings of high cohesion and due to the fact that a single stage makes it possible to remove the pore-formers, both from the precathodic sheet and from the diaphragm, and to provide fresh gel of oxohydroxide of the metal under consideration.

In another preferred alternate embodiment of such process, PTFE is used as a binder for the precathodic sheet and the diaphragm.

In order to further illustrate the present invention and the advantages thereof, the following specific examples are given, it being understood that same are intended only as illustrative and in nowise limitative.

## EXAMPLES

A suspension of the following constituents was prepared with stirring:

- (A) softened water, the amount of which was calculated to provide approximately 4 liters of suspension;
- (B) 100 g of chrysotile asbestos fibers, 200 angstroms in diameter and at least 1 mm in length;
- (C) 1.2 g of octoxynol in the form of a solution in water at a concentration of 40 g/l.

Stirring was carried out for 30 min and then the following various constituents were added in succession, with stirring:

- (D) 25 g of PTFE in the form of a latex containing approximately 65% by weight of solids;
- (E) 30 g of precipitated silica in the form of particles having a mean particle size of 3  $\mu\text{m}$  and whose BET surface area was 250  $\text{m}^2/\text{g}$ ;
- (F) if appropriate, X g of titanium phosphate ( $\alpha$ -TiP), zirconium phosphate ( $\alpha$ -ZrP) or cerium phosphate (CeP) powder;
- (G) 1.5 g of xanthan gum.

Stirring was carried out for 30 min.

The total volume of water was calculated such that the weight percentage of dry solids (B+D+E+F)/A was approximately 4.5%.

The solution was maintained for 48 hours.

The required volume of solution was withdrawn, such that it contained the amount of solids content intended to be deposited to form the diaphragm (on the order of 1.3  $\text{kg}/\text{m}^2$ ).

The suspension was stirred again for 30 min before use.

The filtration was conducted under a programmed vacuum on a bulk cathode (prepared beforehand according to Example 7 of European Patent Application No. 296,076) as follows:

1 min at a vacuum of -5 to -10 mbar relative pressure in relation to atmospheric pressure;  
increasing the vacuum at a rate of 50 mbar/min;  
dewatering for 15 min at maximum vacuum (approximately -800 mbar relative pressure in relation to atmospheric pressure).

The composite was then sintered after optional drying at 100° C. and/or intermediate stabilization of the temperature, by heating the cathode assembly and the diaphragm to 350° C. for 7 min.

The performances of the various composite materials, the production of which was as described immediately above, were then evaluated in an electrolysis cell which exhibited the following characteristics and the operating conditions of which were as indicated below:

Rolled, expanded titanium anode coated with  $\text{TiO}_2$ -  
 $\text{RuO}_2$ ;  
Cathode component made of braided and rolled mild steel; 2 mm wires, 2 mm mesh covered with the precathodic sheet and the diaphragm;  
Anode/cathode component distance: 6 mm;  
Active surface area of the electrolyzer: 0.5  $\text{dm}^2$ ;  
Cell assembled according to the filter press type;  
Current density: 25 A  $\text{dm}^{-2}$   
Temperature: 85° C.  
Operation at constant anode chloride: 4.8 mol  $1^{-1}$ ;

Electrolytic sodium hydroxide concentration: 120 or 200 g/l.

The particular conditions and the results obtained are reported in the Table below:

FY: Faraday yield.

ΔU: voltage at the terminals of the electrolyzer under the specified current density.

Performance (kW h/T Cl<sub>2</sub>)=energy consumption of the system, in kilowatt hours per ton of chlorine produced.

TABLE

| Example No. | Phosphate type | Quantity (g) | Weight deposited 1 g/m <sup>2</sup> | ΔU Volts | FY (%) | NaOH Concentration g/l | Performance kW h/T Cl <sup>2</sup> |
|-------------|----------------|--------------|-------------------------------------|----------|--------|------------------------|------------------------------------|
| 1           | —              | 0            | 1.25                                | 3.13     | 96.5   | 120                    | 2,450                              |
| 2           | α-TiP          | 10           | 1.31                                | 3.18     | 88.5   | 200                    | 2,785                              |
| 3           | α-TiP          | 25           | 1.30                                | 3.13     | 98.5   | 120                    | 2,715                              |
| 4           | α-TiP          | 35           | 1.21                                | 3.35     | 90     | 200                    | 2,400                              |
| 5           | α-ZrP          | 15           | 1.25                                | 3.08     | 86.5   | 200                    | 2,630                              |
| 6           | CeP            | 15           | 1.34                                | 3.20     | 90     | 200                    | 2,785                              |

While the invention has been described in terms of various preferred embodiments, the skilled artisan will appreciate that various modifications, substitutions, omissions, and changes may be made without departing from the spirit thereof. Accordingly, it is intended that the scope of the present invention be limited solely by the scope of the following claims, including equivalents thereof.

What is claimed is:

1. A process for the production of a microporous diaphragm which comprises a sintered, fluoropolymer microconsolidated asbestos-based microporous fibrous sheet material, said sheet material comprising from 3% to 35% by weight of fluoropolymer binder, from 1% to 50% by weight of a uniformly distributed gel of an oxohydroxide of at least one metal of Groups IVA, IVB, VB and VIB of the Periodic Table or of the lanthanide or actinide series thereof, and from 20% to 95% by weight of fibers, at least 1% by weight of said fibers being asbestos fibers, comprising (a) formulating an essentially aqueous dispersion of said fibers, particulates of said fluoropolymer binder and particulates of at least one precursor of an oxohydroxide of at least one metal of Groups IVA, IVB, VB and VIB of the Periodic Table or of the lanthanide or actinide series thereof, (b) depositing a sheet material by vacuum filtering said dispersion through a porous support substrate, (c) removing the liquid material therefrom and optionally drying the sheet material thus formed, (d) sintering said sheet material, (e) formulating a gel from the oxohydroxide precursor of step (a), and (f) treating said sintered sheet material with an aqueous solution of alkali metal hydroxide.

2. The process as defined by claim 1, said porous support substrate comprising a composite cathode component.

3. The process as defined by claim 1, said oxohydroxide precursor comprising a salt selected from the group consisting of α-TiP, α-ZrP and CeP.

4. The process as defined by claim 1, said aqueous dispersion comprising from 5% to 40% by weight of silica.

5. The process for the production of a microporous diaphragm as defined by claim 1, at least 5% by weight of said fibers being asbestos fibers.

6. The process for the production of a microporous diaphragm as defined by claim 1, at least 40% by weight of said fibers being asbestos fibers.

10 7. The process for the production of a microporous

diaphragm as defined by claim 1, comprising a gel of an oxohydroxide of at least one Group IVA and IVB metal.

25 8. The process for the production of a microporous diaphragm as defined by claim 1, comprising a gel selected from the group consisting of titanium, zirconium and cerium oxohydroxide.

30 9. The process for the production of a microporous diaphragm as defined by claim 1, said fluoropolymer binder comprising polytetrafluoroethylene.

35 10. The process for the production of a microporous diaphragm as defined by claim 1, comprising from 1% to 25% by weight of said oxohydroxide gel.

30 11. The process for the production of a microporous diaphragm as defined by claim 1, comprising at least 3% by weight of said oxohydroxide gel.

40 12. The process for the production of a microporous diaphragm as defined by claim 1, said diaphragm comprising fibers selected from the group consisting of fluoropolymer, zirconia, carbon, graphite and titanate fibers.

45 13. The process for the production of a microporous diaphragm as defined by claim 1, weighing from about 0.4 to 3 kg/m<sup>2</sup>.

50 14. A process for the production of a microporous diaphragm comprising (a) formulating an essentially aqueous dispersion of fibers, particulates of a fluoropolymer binder and particulates of at least one precursor of an oxohydroxide of at least one metal of Groups IVA, IVB, VB and VIB of the Periodic Table or of the lanthanide or actinide series thereof, (b) depositing a sheet material by vacuum filtering said dispersion through a porous support substrate, (c) removing a liquid material therefrom and optionally drying the sheet material thus formed, (d) sintering said sheet material, (e) formulating a gel from the oxohydroxide precursor of step (a), and (f) treating said sintered sheet

55 material with an aqueous solution of alkali metal hydroxide.

\* \* \* \* \*